

H. C. EGERTON.  
SHOE SOLE.  
APPLICATION FILED FEB. 23, 1918.  
1,352,730.

Patented Sept. 14, 1920.

Fig. 1,



Fig. 2,



Fig. 3



Fig. 4,



Fig. 5.



Inventor  
Harry C. Egerton  
By his Attorney  
Harry L. Duncan

# UNITED STATES PATENT OFFICE.

HENRY C. EGERTON, OF PASSAIC, NEW JERSEY.

## SHOE-SOLE

1,352,730.

Specification of Letters Patent. Patented Sept. 14, 1920.

Application filed February 23, 1918. Serial No. 218,679.

To all whom it may concern:

Be it known that I, HENRY C. EGERTON, a citizen of the United States, and resident of Passaic, county of Passaic, State of New Jersey, have made a certain new and useful Invention Relating to Shoe-Soles, of which the following is a specification, taken in connection with the accompanying drawing, which forms part of the same.

This invention relates especially to the sole construction of boots and shoes. Ordinary rubber composition soles are objectionable for general use because they are too soft and do not sufficiently resist puncture; bending or penetration when hard objects are stepped upon so that they are often quite objectionable in walking over rough or uneven ground. To obviate these difficulties a sole stiffening element can be provided preferably comprising a plurality of layers of fabric of which one or more outer layers may with advantage be of woven fabric, such as canvas or the like, inclosing, if desired, a more or less thick fibrous center composed of fabric, paper or cotton or other fibrous material, the whole being permanently cemented together with suitable cementing material, which gives the desired strength, stiffness, waterproof and other qualities, such as bakelite or similar phenol aldehyde product, that is phenolic condensation product cementing material. This cementing material can be readily and thoroughly incorporated with the fabric or fibrous material and then the whole cured or hardened by the usual heat treatment so as to form the entire stiffening or reinforcing sheet or element into a single strong and quite rigid unit which can sufficiently reinforce such rubber or other soft shoe soles to make the entire shoe sole structure about as stiff and resistant as an ordinary leather sole. If desired, the surface of the fabric on the bottom of this stiffening element may be suitably coated or provided with a rubber coating and a rubber composition sole and also rubber heel, if desired, may be united therewith by vulcanizing processes at the same time that the phenolic condensation cementing material is cured or hardened to unite the parts of the stiffening sole element. The shoe upper may of course be attached to the rubber sole and stiffening element therefore in any usual or suitable way, whether or not these two sole elements have been pre-

viously vulcanized or otherwise united together, and in some cases especially where the upper is more or less formed of canvas or the like it may be directly molded and cemented by such phenolic condensation cementing material into the sole structure at the same time the parts are united by heat and the rubber sole vulcanized or cured in this connection.

In the accompanying drawing showing in 65 a somewhat diagrammatic way illustrative embodiments of this invention,

Figure 1 is a longitudinal section through a shoe sole and adjacent parts.

Fig. 2 is an enlarged transverse section 70 thereof.

Fig. 3 is a transverse section through a sole stiffening sheet or element.

Fig. 4 is a similar view through one of the modified sole stiffeners; and

Fig. 5 shows still another form of sole stiffener or reinforcing sheet.

As indicated in a rather diagrammatic way in Figs. 1 and 2, the sole stiffening element or sheet may comprise a greater or less 80 number of layers of any suitable fabric, the two outer layers 1 and 2 being preferably of woven fabric such as canvas, for instance, although, of course, finer and thinner fabric may be used in some cases. A fibrous center 85 3 may be interposed between the two outer fabric layers and this center may have varying thickness throughout the different parts of the sole stiffening element, many fibrous materials being suitable for this purpose, 90 such, for example, as flax, jute or cotton fiber in the form, for instance, of cotton batting, fine cotton waste, paper or paper pulp, or mixtures thereof. It is desirable to have greater strength and stiffness at the arch 95 portion of the sole and to secure this additional layers of strengthening fabric 4 may be incorporated at this point in the form of woven fabric or paper which may advantageously be used to some extent at least at 100 this arch portion of the sole where less flexibility is desired. In order to thoroughly incorporate these different materials and form a stiff and strong unitary sole reinforcing element they may be advantageously cemented together by the use of such phenolic condensation material which may be incorporated therewith in any suitable way, as for instance, by more or less impregnating the outer fabric layers and center or other 110

material therewith, or in some cases only parts of these materials may be originally impregnated and the more or less liquid or plastic cementing material forced into or through the others by high pressure when the parts are shaped and molded preparatory to the heat curing or uniting of the parts. It is often desirable to have the stiffening element thinner and softer at the edges, such as 5, so that, if desired, these parts may be readily pierced by the stitching or other uniting means employed for joining the other shoe elements thereto, and for this purpose the outer edges of the sole stiffening sheet or element may advantageously be forced more powerfully together or may have less interposed center material between them, so that this thinner edge portion has also a less proportion of the phenolic condensation cementing material remaining therein which makes it considerably softer and more flexible so as to be more easily penetrated for this purpose. This curing of the phenolic condensation impregnating material may with advantage be what is known in this connection as the moderate curing thereof which may be secured by heating the impregnated material under pressure for an hour or so at a temperature of about 300° Fahrenheit which produces the desired stiffness and strength when the resulting cured sole stiffening element contains 40 to 50 per cent. of the phenolic condensation material.

It is in many cases advantageous to vulcanize the rubber composition sole directly to a sole stiffening fabric or sheet impregnated with or carrying cured phenolic condensation material; and for this purpose one of the outer fabric layers of the stiffening element may be frictioned or coated with rubber composition preferably before it has the phenolic condensation cementing material applied to its other side or incorporated therewith. This lower frictioned or rubber coated surface of the fabric layer 2, for instance, may then be united or forcibly brought into contact with the rubber composition sole 6 formed of the usual rubber sole composition containing, if desired, fibrous material and other filling and wear promoting inert substances, and then the entire sole 6, which may, if desired, include the rubber heel 7, may be united to the sole stiffening element or sheet when the sole is vulcanized by the usual heat treatment therefor which can be carried on at such temperatures and for such times as to properly cure or harden the phenolic condensation cementing material for the sole stiffening element, provided, of course, that the rubber composition is properly selected for this purpose. In this way an integrally united rubber sole and attached stiffening and lining element is produced, such as

shown in Figs. 1 and 2, and this may be stitched or otherwise united to the shoe or boot upper 8 in any suitable way. It is not, however, necessary in all cases to unite these sole elements, and the stiffening and reinforcing sole element or sheet may be built up and cured or permanently united as above described so as to form the separate stiffening or reinforcing sheet shown in section in Fig. 3, which may, of course, extend throughout the entire sole or parts thereof. This preferably has thinner and softer edge portions 5 which for commercial purposes may advantageously be extended so as to leave an edge portion a quarter of an inch or so wide, which may be trimmed off after it has been stitched or otherwise united to the other parts of the shoe and in this way fewer sizes of these stiffening elements can fill the range of commercial requirements. Fig. 4 shows still another illustrative embodiment of the invention in which a heavy canvas or other woven fabric 11 is used on one side of the stiffening element and other suitable fibrous material 12, such, for instance, as a sheet of cotton batting or strong fibrous paper, paper pulp or mixtures thereof in some cases is cemented thereto by the use of such phenolic condensation cementing material which gives the whole the desired stiffness, strength and waterproof properties which are relatively unaffected by the usual heat changes to which footwear is properly subjected. If desired, the woven fabric may extend out to form a thinner or single ply edge 13 which may also in some cases contain relatively smaller proportions of the cementing material so as to be softer and more flexible. Fig. 5 shows still another illustrative form of stiffening element which may be formed of the desired number of plies of canvas or other woven or paper fabric, two plies of heavy cotton duck 14, 15 giving good results for general purposes when something equivalent to eight ounce army duck is used for these two layers. They may be thoroughly and strongly united by first impregnating them with phenolic condensation cementing material of this character and then curing or uniting them by heat after they have been forced directly together so as to preferably give as in the other cases, what is known as the intermediate curing or hardening of such phenolic condensation cementing material, as is known as bakelite varnish. Good results can usually be secured by curing such material under pressure at temperatures of about 300° or so Fahrenheit for an hour or so and when two such layers of duck are cured in this way they can be thoroughly united into a quite hard strong sheet about  $\frac{1}{16}$  of an inch thick which contains some fifty per cent. by weight of the cured phe-

nolic condensation cementing material. The resistance of such a compound sheet stiffening element a sixteenth of an inch thick can be appreciated by considering that a relatively narrow strip can be bent into a circle of two or three inches diameter without cracking or serious injury, and also that the bending modulus of rupture corresponds to 15000 to 18000 pounds or so per square inch. For most purposes where the stiffening element is only used in connection with the front part of the shoe sole and does not extend underneath the entire heel a sixteenth inch sheet of this character has proved to give excellent results under regular service conditions. Of course, it is not necessary that these homogeneous or other stiffening elements shall extend throughout the entire width or area of the sole, and for some purposes, the stiffening element, such as shown in Fig. 5, may be cut somewhat narrower than the shoe sole and may be sewn into the sole structure so as to be entirely concealed by the overlapping edges of the rubber or other sole and upper elements. While, of course, these sole stiffening or reinforcing elements are especially desirable for use with rubber or other soft shoe sole they are naturally not confined thereto and may with advantage be used in connection with regular leather shoe soles and are quite desirable in reinforcing thin or soft leather soles, since they give the necessary stiffness and strength with relatively little weight and cost as compared to leather.

This invention has been described in connection with a number of illustrative embodiments, forms, proportions, elements, parts, shapes, materials, compositions, methods of preparation and use, to the details of which disclosure the invention is not of course to be limited, since what is claimed as new and what is desired to be secured by Letters Patent is set forth in the appended claims:

1. The shoe sole comprising a plurality of layers of woven fabric and additional inner strengthening material including paper adjacent the arch portion of the sole united thereto by cured phenolic condensation cementing material to form an integral sole stiffening member, one side of said outer fabric layers being provided with a rubber coating and a rubber composition sole vulcanized thereto.

2. The shoe sole comprising a layer of woven fabric and additional inner strengthening material including paper united thereto by cured phenolic condensation cementing material and a rubber composition sole.

3. The shoe sole comprising paper fiber material and woven fabric carrying phenolic condensation material and forming an integral sole stiffening element, and a rubber composition sole adhesively united thereto.

4. The shoe sole comprising paper fabric material carrying phenolic condensation material and a composition sole united thereto.

5. The shoe sole element comprising a plurality of layers of paper fiber material carrying and united by cured phenolic condensation cementing material rendering water resistant exposed portions of such fiber material and a rubber composition sole united thereto.

6. The shoe sole element comprising paper fiber material carrying cured phenolic condensation material rendering water resistant exposed portions of such fiber material, and a composition sole element united thereto.

7. The shoe sole stiffening element comprising outer layers of woven fabric containing large proportions of cured incorporated phenolic condensation cementing material and an interposed center comprising unspun fibrous material to space apart the outer layers and strengthen the element, said parts carrying and being united by cured phenolic condensation cementing material to form an integral substantially waterproof element.

8. The shoe sole stiffening element comprising an outer layer of woven fabric containing cured incorporated phenolic condensation cementing material and an interposed center comprising unspun fibrous material to strengthen the element, said parts carrying cured phenolic condensation cementing material to form a substantially waterproof element.

9. The shoe stiffening element comprising an outer layer of fabric containing cured incorporated phenolic condensation cementing material and an interposed center comprising paper fiber material to strengthen the element, said parts carrying cured phenolic condensation cementing material to form a substantially waterproof element.

10. The shaped up shoe stiffening element comprising layers of unspun paper fiber material containing large proportions of cured incorporated phenolic condensation cementing material strengthening and uniting said fibrous material to form an integral substantially waterproof element.

11. The shaped up shoe stiffening element comprising layers of paper fiber material containing large proportions of cured incorporated phenolic condensation cementing material strengthening and uniting said fibrous material to form a substantially waterproof element.

12. The shoe stiffening element comprising layers of paper fiber material containing cured incorporated phenolic condensation cementing material strengthening and uniting said fibrous material to form a substantially waterproof element.

13. The shoe stiffening reinforcing ele-

ment comprising fabric and additional paper fibrous material, said materials being united by incorporated cured phenolic condensation cementing material to form an integral shoe stiffening element.

14. The footwear stiffening element comprising paper carrying incorporated cured phenolic condensation cementing material to form an integral water resistant stiffening element.

15. The shoe stiffening element comprising a body of paper fiber material and an outer woven fabric layer carrying and united to said body by impregnating cured phenolic condensation cementing material

stiffening and strengthening the element and rendering such outer fabrics substantially waterproof.

16. The shoe stiffening element comprising paper fiber material united and impregnated by cured phenolic cementing material to form an integral water resistant element.

17. The shoe stiffening element comprising paper fiber material carrying phenolic cementing material.

HENRY C. EGERTON.

Witnesses:

HARRY L. DUNCAN,  
JESSIE B. KAY.